

## UNITED STATES PATENT OFFICE

2,243,054

DETERGENT COMPOSITION AND  
MANUFACTURE THEREOF

James G. Vail, Media, Pa., assignor to Philadelphia Quartz Company, Philadelphia, Pa., a corporation of Pennsylvania

No Drawing. Application November 27, 1937,  
Serial No. 176,931

7 Claims. (Cl. 252—109)

This invention relates to manufacture of detergent compositions; and it comprises a process wherein finely divided particles of an expanded alkali metal silicate, usually containing not substantially less than one mole of alkali metal oxide to two moles of silica, are reacted with a fatty acid in the substantial absence of water under conditions forming an alkali metal soap, the specific surface of the particles of the alkali metal silicate being such that a substantially homogenous product is formed, and the proportions of alkali metal silicate and of fatty acid being such that the final product contains at least about 5 per cent of soap and a substantial proportion of alkali metal silicate, advantageously having a molecular ratio of alkali metal oxide to  $\text{SiO}_2$  ranging from about 1:1.5 to 1:3.3. My invention also includes the detergent composition formed as a result of the described process, this detergent comprising particles of an alkali metal silicate substantially uniformly combined with at least about 5 per cent of an alkali metal soap formed in situ by reaction of said particles of alkali metal silicate with a fatty acid, said particles containing alkali metal silicate, advantageously having a molecular ratio of alkali metal oxide to  $\text{SiO}_2$  ranging from about 1:1.5 to 1:3.3; all as more fully herein-after set forth and as claimed.

The field of detergents is one of the most ancient of the chemical arts. Fats and fatty oils have been saponified with alkalis of all types and it has long been known, for example, that soaps can be made by the use of alkali metal silicates as saponifying agents. It has also long been known that fatty acids can be substituted for the fats and fatty oils in the manufacture of soaps. Alkali metal silicates have been used not only as saponifying agents but also as builders for soaps and it has been definitely established that the presence of alkali metal silicates substantially increases the detergency of soaps with which they are mixed. But no entirely satisfactory commercial process has as yet been proposed for incorporating alkali metal silicates in soaps in the desired proportions.

The usual process of making silicated soaps is to crutch, that is, to mix a hot kettle soap with a silicate solution at a temperature in the neighborhood of 140° F. until an apparently homogeneous mass is produced. The resulting mixture, which is poured into frames to cool at this stage, is not at equilibrium, however, and always exhibits more or less tendency for the silicate solution to separate in the frames. Separation

may be avoided by cooling the frames as quickly as may be convenient, thus increasing the viscosity and in effect producing a frozen heterogeneous mixture. This process is time consuming and has rather severe limitations since the soap and silicate are not miscible in all proportions and the more siliceous silicates are likely to take up alkali from the soap, resulting in a grainy condition. If the product is made in the form of bars, the amount of silicate which can be added is limited by the shrinkage of the bar soap upon drying and also due to the fact that a highly silicated soap hardens and becomes difficultly soluble upon ageing.

15. Spray dried mixtures of silicates and soap are manufactured by spraying a fluid mixture into a current of hot air, this operation causing the evaporation of much of the water present and producing a product in the form of small bubbles, having a high specific volume and ready solubility. A substantial amount of water is evaporated during the spray drying process. Spray cooling processes are also known for making mixtures of silicates and soap. In these processes it is necessary to add roughly 20 per cent of sodium carbonate which eliminates the necessity for evaporating the water present. But the product thus formed is not as desirable from a detergent viewpoint. Both of these processes are difficult to control and are costly. In the present process evaporation of the water is entirely avoided and it is not necessary to add extraneous salts.

35. I have found that solid alkali metal silicates will react readily and to substantial completion with fatty acids of high molecular weight in the substantial absence of water to form a homogeneous product, provided that the physical state of the alkali silicate is such as to expose a large surface area per unit of volume, that is provided that its specific surface (surface divided by volume) is sufficiently large or that its apparent specific gravity is sufficiently low, i. e. provided that expanded silicates are employed.

40. This process is characterized by the fact that, unless the particles of alkali metal silicate are disrupted during the reaction, by grinding, for example, the particles of the resultant product are substantially determined by the physical characteristics of the particles of the silicate used in the process. If a so-called intumescent silicate is employed, having an apparent specific gravity of the order of 0.1, for example, the specific gravity of the resulting product may be increased to about 0.3, but this product otherwise

possesses most of the physical characteristics of the silicate from which it was made. Even the shapes of the silicate particles are retained. The mechanism of my reaction thus appears to be a saponification which proceeds from the interface between the silicate and the fatty acid, resulting in the formation of a solid soap in apparently homogeneous relation to the silicate which may be present in large amounts, the soap being formed on the alkali nuclei by accretion but penetrating to the cores of the particles, that is, completely through the silicate. This enables my product to be identified and distinguished from products of similar composition produced by other methods.

The reaction between the alkali silicate and the fatty acid in my process can be conducted at temperatures ranging from room temperatures to temperatures approaching those at which the fatty acid is decomposed or volatilized. Temperatures above the melting points of the fatty acids are advantageous. One important advantage of my process is that temperatures substantially below those causing damage to the fatty acid can be employed. At the lower temperatures, if an anhydrous silicate is used, it is desirable to add a small amount of water to the process since otherwise the reaction is time consuming. The amount of water required, however, amounts to only about 1 to 10 per cent by weight, based on the weight of the mixture. When a hydrated silicate is employed the addition of water is not required. It will be noted that one molecule of water is formed during the chemical reaction involved in my process and this may account for the small amount of water required to initiate the reaction. At higher temperatures my process proceeds at a satisfactory rate even in the absence of added water and with the use of anhydrous silicates, these products usually containing sufficient water to initiate the reaction or absorbing such water during the process. It is thus seen that the amount of water desired in the final product can be accurately predetermined by the addition of the required amount during the process. A certain amount of water is usually desired in my detergents since this makes the products more readily soluble.

I have found that the use of the so-called intumescent silicates is particularly advantageous in my process. These silicates are formed by rapidly heating hydrated silicates to expel part of the water in the form of bubbles which expand as they are released from the surface of the more-or-less plastic silicate, resulting in a highly porous product of very low apparent specific gravity. Advantageous results have also been obtained by using flaked silicates produced by the rotation of cooled drums in heated, concentrated silicate solutions, followed by scraping the resulting films of silicate from the drums. These flaked silicates also have very low apparent specific gravities and large specific surfaces. Spray dried silicates of low apparent specific gravity are suitable for use in my process. All other silicates having similar physical properties can be used in my process. The term "expanded silicates" can be applied to these products.

There are various ways in which my reaction may be conducted. It is only necessary to uniformly mix the fatty acid with the particles of silicate in such manner that these particles are uniformly coated. This can be accomplished, for example, by spraying a heated fatty acid over the silicate while the latter is being agitated, or by

adding the fatty acid in solid form to a mixer which is heated. When a liquid fatty acid is employed, mixing may be accomplished by the use of an ordinary rotary drum. If desired the solid silicate can be added gradually to the liquid fatty acid and this mixture agitated until the desired granular product is obtained. When a flaked silicate is employed the process of flaking and mixing can be combined by spraying the fatty acid over the film of silicate formed on the rotating drum prior to the scrapers. The silicate and fatty acid can be ground together during the reaction if desired. A considerable amount of heat is given off during the reaction.

If the product is to be stored prior to use, the silicate particles can be coated with fatty acid in the cold and the reaction allowed to proceed to completion during storage. It is more advantageous, however, to heat the mixture of fatty acid and silicate while mixing is taking place in order to produce a homogeneous and stable product. The temperatures required depend upon the fatty acid employed. For stearic acid, for example, temperatures ranging from about 60° to 90° C. are suitable, the reaction requiring from about 30 to 50 minutes, this time depending upon the fineness of the silicate and the amount of water in the system. A stable product thus results, which remains loose and free flowing in storage.

It is seen from the above that my process produces a product which is stable and homogeneous and which possesses the greatly desired characteristics of rapid solubility, and lightness in weight. This process is capable of producing compositions containing widely varying ratios of soap to silicate and also widely different ratios of alkali metal oxide to silica in the silicate component of the product. It should also be mentioned that my reaction goes to substantial completion which is in contrast to the process in which fatty acids are reacted with sodium carbonate, for example, which process is incomplete and requires the addition of caustic soda in order that the fatty acid should be completely saponified.

It is possible, of course, to add other detergent salts during my process. Examples of suitable salts are sodium carbonate and phosphates, which may be added in the form of their solutions, if desired. These salts appear in the final product in more-or-less unchanged form. They are not required in the product, however, and in some cases are not desired.

The following specific examples illustrate certain processes which are within the scope of the present invention and which represent practical methods of making my novel products.

#### Example 1

56.7 parts stearic acid were melted in a mixer and agitated at about 70° C. 33.3 parts of anhydrous crystalline metasilicate ( $Na_2SiO_3$ )—65 mesh—were added, this product having an apparent specific gravity of about 0.7. 10 parts of water were also added. The mass gradually thickened as the individual grains appeared to grow in size. Strong, slow agitation was continued until the batch assumed a granular character and no liquid oil was visible. It was then allowed to cool. The product had an apparent density of about 0.7.

#### Example 2

100 parts of expanded  $Na_2O \cdot 2SiO_2$  containing 14 per cent water and an apparent density of

about .04 were agitated by rolling in a drum at about 25° C. Oleic acid, 100 parts were distributed over the moving mass which remained solid throughout the process, but lost its apparent oiliness as the reaction proceeded. The temperature rose to about 45° C. and the final product had an apparent density of .18. A similar product was made with melted stearic acid at about 70° C. This had an apparent density of 0.2.

Such products made with red oil are soluble in cold water, while hot water is necessary to dissolve the products made from stearic acid.

While I have described what I consider to be the more advantageous embodiments of my process, it is evident that many modifications can be made in the specific procedures which have been described, without departing from the purview of this invention. As mentioned previously, it is merely necessary to thoroughly mix a soap-forming fatty acid with a solid expanded silicate in suitable proportions to produce the desired reaction, this reaction usually taking place even in the absence of added water. When water is added, this may be accomplished by the addition of a suitable solution of an alkali metal silicate or of another salt, the water thus added appearing in the final product and tending to make the latter more readily soluble. The addition of silicate solutions as sources of water for the reaction is a useful means of regulating the ratio of alkali to silica in the finished product. Any soap-forming fatty acid can be used in my process, oleic and stearic acids being chosen to illustrate high and low melting points. The fatty acids used in the process may be dissolved in a suitable solvent, such as petroleum ether, prior to or during their admixture with the silicate, if desired. The silicates of various alkali metals can be employed. For example, expanded potassium silicates can be used in place of sodium silicates and are capable of producing very similar products. While I prefer to employ solid silicates having apparent specific gravities ranging up to about 0.7, somewhat more dense products can be employed provided that a longer time is allowed for the reaction to take place. The lighter weight silicates produce lighter weight products if the same amounts of fatty acid are added, and the lighter weight products are usually more advantageous. It is possible to produce products having apparent specific gravities as low as about 0.1, for example, this value rising to about 0.9 when the heavier silicates are employed. Intumescent silicates having apparent specific gravities as low as about 0.01 can be produced and are useful in my process. The resulting products have little tendency to produce dust. I have also subjected spray dried silicates to a rapid heating to produce intumescence, thus obtaining an extremely light-weight silicate for use in my process. While my process can be varied in such manner that the residual alkali metal silicate in the product has a rather wide range of molecular ratios of Na<sub>2</sub>O to SiO<sub>2</sub>, the more advantageous detergents within this invention contain silicates wherein this ratio lies between about 1:1.5 and 1:3.3. It has been found that the particles of my detergents usually contain somewhat higher proportions of soap on the surface than in the interior which serves to

distinguish my products from the usual silicated-soap products. This difference is so slight, however, that the products can be called substantially homogeneous. Other modifications of my process which fall within the scope of the following claims will be immediately evident to those skilled in the art.

What I claim is:

1. As a new detergent, particles of an expanded alkali metal silicate substantially uniformly combined with at least about 5 per cent of an alkali metal soap formed in situ by reaction of said particles of alkali metal silicate with a high molecular fatty acid, said particles containing slightly larger proportions of soap on their surfaces than in their interiors, said detergent having an apparent specific gravity between about 0.1 and 0.9.
2. The product of claim 1 wherein the alkali metal silicate component contains alkali metal oxide and SiO<sub>2</sub> in a molecular ratio ranging from about 1:1.5 to 1:3.3.
3. The product of claim 1 wherein the alkali metal silicate component is sodium silicate containing Na<sub>2</sub>O and SiO<sub>2</sub> in a molecular ratio varying from about 1:1.5 to 1:3.3.
4. As a new detergent, intumescent particles of a sodium silicate substantially uniformly combined with at least about 5 per cent of a sodium soap but containing on their surfaces slightly larger proportions of soap than in their interiors, said particles having an apparent specific gravity ranging from about 0.1 to 0.9, said sodium soap resulting from the reaction of a high-molecular fatty acid with said intumescent particles of sodium silicate.
5. The product of claim 4 containing sufficient water to make it readily soluble.
6. As a new detergent, expanded particles of a sodium silicate substantially uniformly combined with at least about 5 per cent of a sodium soap formed in situ by reaction of said particles with a high-molecular fatty acid, the sodium silicate in said product containing Na<sub>2</sub>O and SiO<sub>2</sub> in a ratio varying from about 1:1.5 to 1:3.3 and the apparent specific gravity of said product varying from about 0.1 to 0.9.
7. In the manufacture of detergents, the process which comprises slowly agitating granular particles of an expanded sodium silicate, having an apparent specific gravity not substantially exceeding 0.7 and having a molecular ratio of Na<sub>2</sub>O to SiO<sub>2</sub> within the range of about 1:1.5 to 1:3.3, in the presence of liquid, soap-forming fatty acid in amount sufficient to form at least about 5 per cent of soap in the final product and continuing the slow agitation without substantial disintegration of the silicate particles until no liquid fatty acid is visible and a granular product is produced, whereby soap is formed by accretion on the silicate particles, the resulting silicate-soap particles being of substantially uniform composition but having a slightly larger proportion of soap on their surfaces than at their cores, having the general form and physical characteristics of the original silicate particles and having an apparent specific gravity not substantially exceeding 0.9.

JAMES G. VAIL.